



US005625858A

## United States Patent [19]

Hirai et al.

[11] Patent Number: 5,625,858

[45] Date of Patent: Apr. 29, 1997

[54] CONTACT CHARGING MEMBER, PROCESS FOR PRODUCING SAME AND ELECTROPHOTOGRAPHIC APPARATUS USING SAME

[75] Inventors: Yoshihiro Hirai, Ibaraki-ken; Takashi Yamashita, Nagareyama; Masaaki Takenaka, Kashiwa, all of Japan

[73] Assignees: Canon Kabushiki Kaisha, Tokyo; Canon Kasei Kabushiki Kaisha, Ibaraki-ken, both of Japan

[21] Appl. No.: 586,091

[22] Filed: Jan. 16, 1996

[30] Foreign Application Priority Data

Jan. 18, 1995 [JP] Japan 7-005729

[51] Int. Cl. <sup>6</sup> G03G 15/02

[52] U.S. Cl. 399/176; 492/56

[58] Field of Search 355/219; 361/225; 492/56; 29/895.212, 895.32

[56] References Cited

U.S. PATENT DOCUMENTS

5,567,494 10/1996 Ageishi et al. 355/219 X

FOREIGN PATENT DOCUMENTS

|           |        |       |
|-----------|--------|-------|
| 56-104349 | 8/1981 | Japan |
| 63-167380 | 3/1988 | Japan |
| 64-24264  | 1/1989 | Japan |
| 3-59682   | 3/1991 | Japan |
| 5-2313    | 1/1993 | Japan |

Primary Examiner—Joan H. Pendegrass  
Attorney, Agent, or Firm—Fitzpatrick, Cella, Harper & Scinto

[57] ABSTRACT

A contact charging member to be abutted against a charge-receiving member and supplied with a voltage for charging the charge-receiving member is provided. The charging member includes an electroconductive substrate, an elastic layer and a surface layer disposed in lamination. The surface layer comprises crosslinked polymer crosslinked by irradiation with an electron beam. The surface layer may preferably be in the form of a seamless tube formed of the crosslinked polymer. The surface layer crosslinked by electron beam irradiation is less liable to suffer from transfer of a crosslinking agent or a decomposition product thereof to the charge-receiving member. Accordingly, the charging member shows improved durability and stably uniform charging ability suitable for electrophotographic image formation under various environmental conditions.

16 Claims, 2 Drawing Sheets





FIG. 1



FIG. 2

**CONTACT CHARGING MEMBER, PROCESS  
FOR PRODUCING SAME AND  
ELECTROPHOTOGRAPHIC APPARATUS  
USING SAME**

**FIELD OF THE INVENTION AND RELATED  
ART**

The present invention relates to a charging member for charging a charge-receiving member (a member to be charged) in contact with the charge-receiving member, a process for production thereof and an electrophotographic apparatus using the charging member.

In an image forming apparatus including an electrophotographic apparatus (such as a copying machine or a printer) and an electrostatic recording apparatus, a corona discharger has principally been used heretofore, as means for non-contactively charging the surface of an image-carrying member as a charge-receiving member including a photo-sensitive member, a dielectric material, etc. Such a corona discharger has an advantage of excellent uniform charging ability.

However, the corona discharger requires an expensive high-voltage power supply and a space for, e.g., shielding itself or the high-voltage power supply. Further, it is accomplished with occurrence of relatively much corona-discharge by-products, such as ozone, so that it also requires auxiliary means and mechanism for dealing with the by-products, thus resulting in an increase in size and production cost of the apparatus.

For such reasons, a charging means of the contact charging-type has been increasingly adopted. The contact charging is a process for charging a charge-receiving member surface to prescribed polarity and voltage by causing a charging member under application of a voltage to contact the charge-receiving member, and is accompanied with advantages, such as a lower voltage of power supply, little occurrence of by-products, such as ozone, as encountered in corona-discharging, and a simpler cost leading to a lower production cost.

Depending on the shape and form of the charging member used, the contact charging device may be classified into a roller-type charger using a charging member in the form of a roller (charging roller) (as disclosed in, e.g., Japanese Laid-Open Patent Application (JP-A) 63-167380 and JP-A 56-91253); a blade-type charger including a blade-shaped member (charging blade) (as disclosed in, e.g., JP-A 64-24264 and JP-A 56-104349), and a brush-type charger including a brush-shaped member (as disclosed, e.g., in JP-A 64-24264).

The charging member can be supplied with a DC voltage alone (DC voltage application scheme), but may preferably be subjected to a scheme (AC voltage application scheme) wherein a charge-receiving member is charged by forming an oscillating electric field (alternating electric field or AC electric field, e.g., an electric field or voltage of which the voltage value periodically changes with time) having a peak-to-peak voltage which is at least two times a charging initiation voltage of the charge-receiving member at the time of applying DC voltages to the contact charging member, because it is possible to effect a uniform charging treatment.

The charging roller in the roller-type charger is rotatably held about an axis and is pressed against the charge-receiving member surface at a prescribed pressure so as to rotate following the movement of the charge-receiving member surface.

The charging roller ordinarily has a multi-layer structure comprising a core metal at the center, an electroconductive

elastic layer in the form of a roller disposed to surround the core metal, and a surface layer disposed on the outer peripheral surface thereof.

In the above structure, the core metal is a rigid body for retaining the entire shape of a roller and also functions as an electricity-supplying electrode layer.

The elastic layer ordinarily comprises an electroconductive member having a volume resistivity of  $10^4$ – $10^9$  ohm.cm and also has a function of ensuring a uniform contact with the charge-receiving member surface through its elastic deformation. Accordingly, the elastic layer ordinarily comprises a vulcanized rubber having a resiliency as represented by a rubber hardness (JIS A) of at most 70 degrees.

The surface layer has functions of improving the uniform chargeability of the charge-receiving member, preventing the occurrence of leakage attributable to pinholes, etc., on the charge-receiving member surface, preventing the sticking of toner particles or paper dust and preventing the bleeding out of oil or a plasticizer added to the elastic layer for lowering the hardness thereof. The surface layer may have a volume resistivity of  $10^5$ – $10^{13}$  ohm.cm and has been conventionally formed by applying an electroconductive paint.

Further, in view of the condition for use thereof, the charging member is required to be surfaced with a material having good mechanical strength, wear resistance, ozone resistance, and heat and cold resistance, and having a low moisture-absorptivity, a good resiliency, a creep resistance, a low compression permanent strain and an easy processability.

If the surfacing material does not satisfy the above-mentioned properties, the charging roller is liable to deteriorate during the use or cannot fit to a change in-environmental condition to result in image defects.

Further, in case where an oscillating electric field is formed between the charger and the charge-receiving member so as to effect the uniform charging of the charge-receiving member, it is possible that a mechanical oscillation is induced therebetween to cause an abnormal sound, which may be called a charging sound and the suppression of which has imposed an important problem.

The charging sound may be effectively reduced by lowering the rubber hardness of the elastic layer, but it is difficult to accomplish a sufficient lowering in hardness by simply increasing the amount of the softening agent. Accordingly, it has been considered to use a rubber foam or a spongy rubber. The thus-formed charging roller may be referred to as a foam-type charging roller, and another type using no foam material may be referred to as a solid-type charging roller.

In the case of a foam-type charging roller, a surface skin layer formed at the time of vulcanization is liable to have a poor surface smoothness, so that the skin layer has to be removed by an abrasion treatment. However, as the uniformization of a bubble or cell size is difficult, a large size of bubble is liable to be exposed at the surface by the abrasion, resulting in a concavity in the surface layer formed by application in the subsequent step. Such a surface concavity formed in the surface layer of a charging roller results in a charging failure and fails in providing good images.

On the other hand, there has been proposed a method wherein a polymeric material is preliminarily formed into a seamless tube and is then used to cover an elastic layer to form a surface layer (JP-A 3-59682 and JP-A 5-2313).

In the case of using a seamless tube described above, the resultant surface layer can be free from a concavity even if

the elastic layer therebelow is accompanied with a large bubble, thus providing a charging roller excellent in surface smoothness. However, the surface layer also has many functions as described above, so that it is also required to have excellent mechanical strength, wear resistance, ozone resistance and hot-and-cold resistance.

#### SUMMARY OF THE INVENTION

A generic object of the present invention is to provide a contact charging member excellent in physical properties as described above.

Another object of the present invention is to provide a process for producing such a contact charging member.

A further object of the present invention is to provide an electrophotographic apparatus using such a contact charging member.

According to the present invention, there is provided a contact charging member to be abutted against a charge-receiving member and supplied with a voltage for charging the charge-receiving member, comprising an electroconductive substrate, an elastic layer and a surface layer disposed in lamination; said surface layer comprising a crosslinked polymer crosslinked by irradiation with an electron beam.

According to another aspect of the present invention, there is also provided a process for producing a contact charging member to be abutted against a charge-receiving member and supplied with a voltage for charging the charge-receiving member, comprising the steps of:

- (1) forming an elastic layer on an electroconductive substrate,
- (2) shaping a polymer into a seamless tube,
- (3) crosslinking the polymer in the shape of the seamless tube by irradiation with an electron beam, and
- (4) covering the elastic layer with the crosslinked seamless tube.

According to a further aspect of the present invention, there are provided an electrophotographic apparatus and a process cartridge for such an electrophotographic apparatus, respectively including a contact charging member as described above.

These and other objects, features and advantages of the present invention will become more apparent upon a consideration of the following description of the preferred embodiments of the present invention taken in conjunction with the accompanying drawings.

#### BRIEF DESCRIPTION OF THE DRAWINGS

FIG. 1 is a schematic illustration of a transfer-type electrophotographic apparatus including a contact charging member according to the invention.

FIG. 2 is an illustration of an electron beam irradiation apparatus suitably used in the invention.

#### DETAILED DESCRIPTION OF THE INVENTION

The elastic layer constituting the contact charging member according to the present invention may comprise an electroconductive rubber composition principally comprising an elastic material and a conductivity-imparting agent.

The elastic material may appropriately comprise: a rubber, such as silicone rubber, ethylene-propylene rubber, EPDM (ethyl/propyl/diene terpolymer) fluorinated rubber, urethane rubber, epichlorohydrin rubber, epichlorohydrin-ethylene oxide rubber, acrylic rubber, ethylene-acrylic

rubber, natural rubber, isoprene rubber, butadiene rubber, 1,2-polybutadiene, styrene-butadiene rubber, chloroprene rubber, nitrile rubber, modified nitrile rubber, butyl rubber, chlorosulfonated polyethylene rubber, polysulfide rubber, or 5 chlorinated polyethylene rubber; or a thermoplastic elastomer of styrene-type, olefin-type, ester-type, urethane-type, isoprene-type, 1,2-butadiene-type, vinyl chloride-type, amide-type, ionomer-type, etc.

The conductivity-imparting material for imparting an 10 electroconductivity to the elastic layer may comprise a known material. Examples thereof may include: carbon fine particles inclusive of carbon black and graphite particles; fine particles of metals, such as nickel, silver, aluminum, and copper; fine particles composed principally of metal oxides, 15 such as tin oxide, zinc oxide, titanium oxide, aluminum oxide and silica, doped with impurity ions having different atomic valences; electroconductive fiber such as carbon fiber, fiber of metal such as stainless steel, electroconductive whisker, such as carbon whisker and electroconductive 20 potassium titanate whisker obtained surface-treating potassium titanate whisker with a metal oxide, carbon, etc., for electroconductivity imparting; and fine particles of electroconductive polymers, such as polyaniline and polypyrrole.

The elastic layer containing a conductivity-imparting 25 material may ordinarily be formed adjacent to a core metal as an electroconductive substrate or electricity-supplying electrode (layer) to assume a shape of roller. Hereinafter, such a core metal and elastic layer may be integrally called a roller member.

30 The elastic layer may be formed through processes which are not particularly restricted but may be ordinary rubber-shaping process, such as injection molding, extrusion and press-forming. The core and the elastic layer may be integrated with each other by directly forming the elastic layer 35 surrounding the core metal by the insert molding process or by shaping the elastic layer in the form of a thick tube and inserting the core metal into the thick tube.

It is possible to reduce the rigidity of the elastic layer by 40 incorporating a softening agent, such as an oil or plasticizer, in the above-mentioned electroconductive rubber composition. As another method, the rigidity of the elastic layer may be reduced by forming the elastic layer of a rubber foam.

It is important that the elastic layer has a macroscopically 45 smooth surface. Accordingly, in case where the elastic layer does not have a sufficiently smooth surface after its formation, e.g., when it is formed as a rubber foam or with a spew line as by the press forming process, a secondary smoothening treatment as by abrasion or trimming may be 50 required.

Further, as the elastic layer is ordinarily pressed against the charge-receiving member, it is desired that the elastic layer has small compression permanent strain. Accordingly, the elastic layer may desirably be formed of a vulcanized 55 rubber or a crosslinked rubber.

The polymer constituting the surface layer of the contact 60 charging member according to the present invention may suitably comprise various rubbers or thermoplastic elastomers as described above for constituting the elastic layer.

65 The polymer may also be a plastic material, examples of which may include: polyolefins, such as polyethylene, ethylene copolymers, polypropylene, propylene/ethylene copolymer, polybutene, and poly-4-methyl-pentene-1; polyamides, such as nylon 6, nylon 66, nylon 11, nylon 12 and other copolymer nylons; saturated polyesters, such as PET (polyethylene terephthalate) and PBT (polybutylene terephthalate); polycarbonate; styrene-type resins, such as

polystyrene, HIPS (high-impact polystyrene), ABS (acrylonitrile/butadiene/styrene copolymer), AES (acrylonitrile/EPDM/styrene), and AAS (acrylonitrile/acrylate/styrene); acrylic resins; vinyl chloride resins; vinylidene chloride resins; polyacetal; polyphenylene oxide and polystyrene-modified products thereof; polyimide resins; polyallylate; and vinylidene fluoride homopolymers and copolymers. It is further possible to use a polymer alloy or a polymer blend including two or more species of polymers, selected from the above-mentioned rubbers, thermoplastic elastomers and plastic materials.

The surface layer can be formed by applying such a crosslinkable polymer onto the elastic layer surface and irradiating the polymer layer with an electron beam or electron rays to cause crosslinking reaction.

The surface layer may also be formed by first shaping such a polymer into a seamless tube and then covering the elastic layer with the seamless tube of the polymer. More specifically, the seamless tube may be prepared by subjecting a polymer comprising such a polymer, a conductivity imparting agent as described above and another optional additive, as desired, to the extrusion forming, the injection molding, the blow forming, etc., to form a tube of the composition. Among the above, the extrusion forming is particularly suited.

The polymer layer or tube simply formed according to the forming or shaping process described above cannot sufficiently satisfy the properties required for the surface layer or the surface layer material. Accordingly, the polymer is crosslinked by irradiation with an electron beam or electron rays. For the crosslinking, there has been known the chemical crosslinking process wherein a crosslinking agent, such as sulfur, an organic peroxide or an amine, appropriately selected depending on the polymer, is added to the polymer composition, and then the polymer composition is heated. The electron beam crosslinking is advantageous than the chemical crosslinking process because it requires no or less crosslinking agent and is less liable to of soil the charge-receiving member with the crosslinking agent or decomposition products thereof and no requirement for high-temperature treatment, and than the  $\gamma$ -ray crosslinking because of the safety of the process.

The crosslinked polymer thus-obtained may be provided with improved wear resistance, heat resistance and anti-creep characteristic compared with the corresponding non-crosslinked polymer, thus being expected to satisfy the properties required of the surface layer.

A representative structure of an electron beam irradiation apparatus suitably used for crosslinking in the present invention may be one as shown in FIG. 1. Referring to FIG. 2, an electric power is supplied from a DC power supply 20 via a cable 21 to an accelerating pipe 22, where hot electrons issued from a high-temperature metal filament are accelerated under an accelerating voltage of 150-1000 kV to form a spotty electron beam. The electron beam is supplied with a high-frequency magnetic field, when it passes through a scanner, to form a scanning electron beam, which is then omitted through a window to irradiate an object to be crosslinked, i.e., a polymer tube or coating, disposed directly below the window.

The crosslinking by electron beam irradiation may be effected at various points of time during the tube formation. More specifically, the crosslinking may be effected either after the tube formation and before the insertion of a roller member, or after the insertion of a roller member. Further, in the case of forming the surface layer by wet coating, it is

generally preferred to once dry the polymer coating film and then irradiate the coating film with an electron beam.

In the electron beam crosslinking process, it is sometimes desirable to add a crosslinking aid depending on the species of a polymer to be crosslinked so as to provide the crosslinked polymer with improved physical properties.

Preferred examples of the crosslinking aid may include polyfunctional monomers, such as triallyl isocyanurate, tetra-<sup>10</sup>raethylene glycol dimethacrylate, divinylbenzene, diallyl phthalate, trimethylolpropane, trimethacrylate, trimethylpropane triacrylate, triallyl cyanurate, tetramethylolmethane tetramethacrylate, and trimethoxyethoxyvinylsilane.

Ordinarily, the irradiation dose may suitably be in the range of 5-50 Mrad (corresponding to 12 to 120 calorie per gram of the polymer) but may be selected at an appropriate level depending on factors, such as the species of a polymer the presence or absence of a crosslinking aid and the accelerating voltage level.

The crosslinking seamless tube may preferably have a thickness of 100-500  $\mu$ m, more preferably 150-350  $\mu$ m.

On the other hand, the surface layer prepared through the wet coating process may suitably have a thickness of 10-150  $\mu$ m.

The surface layer in its state after being finished into the surface layer of the charging member may preferably have a resistivity of  $10^5$ - $10^{13}$  ohm.cm, particularly  $10^6$ - $10^{12}$  ohm.cm.

As described above, a seamless tube for constituting the surface layer may suitably be formed by extrusion. More specifically, the polymer, the electroconductivity-imparting agent and another optional additive, such as a crosslinking agent and/or stabilizer are formulated into a compound in advance, which compound is then knead and extruded by an extruder and extruded through a die having a ring-shaped slit, followed by cooling to continuously form a seamless tube.

A heat-shrinkable tube may be prepared if the tube size is enlarged, e.g., by air-pressurization during the cooling or re-heating after the cooling, or a non-heat-shrinkable tube may be prepared if such a size-enlarging treatment is not applied.

The seamless tube used in the present invention may be either non-heat-shrinkable or heat-shrinkable but can be used to cover the elastic layer in different manners depending on whether it is either of the two.

In the case of a non-heat-shrinkable tube, the tube is required to have an inner diameter which is at most the outer diameter of the elastic layer so as to ensure an intimate attachment between the elastic layer and the surface layer and, while the tube diameter is enlarged by blowing a compressed air, the roller member is inserted into the tube, followed by releasing the air pressure to complete the insertion or coverage with the tube.

On the other hand, in the case of a heat-shrinkable tube, the tube may desirably have an inner diameter larger than the outer diameter of the elastic layer and, after being inserted with the roller member, are caused to thermally shrink about the elastic layer to effect an intimate attachment, e.g., by heating for a prescribed period in a thermostat vessel held at a temperature in the vicinity of the softening point thereof, to complete the insertion or coverage of the roller member.

Next, a further description is added regarding respective polymers.

Polyethylene, which is ordinarily a homopolymer of ethylene, may be classified into low-density polyethylene or

high-density polyethylene depending on a different degree of crystallization. As a special grade, it is also possible to use a copolymer of ethylene with a polar polymer, examples of which may include vinyl acetate, acrylic monomer such as methyl methacrylate or acrylic acid, maleic anhydride, vinyl chloride and vinylsilane. In recent years, a copolymer with  $\alpha$ -olefin, such as 1-butene (linear low-density polyethylene) has also been used. Herein, the above-mentioned homopolymer and copolymers of ethylene may be included in polyethylene.

Polyethylene has many excellent properties but has a poor heat resistance so that, when it is used to constitute a surface layer of a charging roller in its uncrosslinked state, the resultant surface layer deforms due to creep, thus losing its surface smoothness.

In addition to the above-mentioned conductivity-imparting agent, the crosslinked polyethylene can further contain various optional additives, such as a stabilizer, a lubricant and insulating fillers, as desired.

Polyamides may include nylon 12 which is generally produced by polycondensation of  $\omega$ -laurolactam or 12-aminodecanoic acid, and nylon 11 which is generally produced by polycondensation of 11-aminoundecanoic acid.

The above-mentioned two species of polyamides, i.e., nylon 12 and nylon 11, have remarkably different molecular structures compared with general purpose polyamides, such as nylon 6 and nylon 66, and are excellent in softness, wear resistance and low-temperature property and have low moisture-absorptivity, which are suited for constituting the surface layer of a charging member.

To the nylon 12 or nylon 11, it is possible to add various stabilizers and insulating fillers, as desired, in addition to the above-mentioned charge-imparting agent.

The electron beam curing of a polyamide may be promoted by preliminary addition of an allyl compound such as triallyl isocyanurate, so as to allow effective crosslinking by electron beam irradiation in air.

Ethylene-acrylic rubber, which is a relatively novel rubber first commercialized by E. I. Dupont in 1975, may be regarded as a type of acrylic rubber in a broad sense but has a significant difference in molecular structure from ordinary acrylic rubber and correspondingly has remarkably characteristic physical properties.

The ethylene-acrylic rubber principally comprise a binary copolymer of ethylene and methyl acrylate and is ordinarily commercially available as a ternary copolymer including a carboxylic compound as a third monomer. The ethylene-acrylic rubber may be either a binary or ternary copolymer as described above.

The ethylene-acrylic rubber has advantageous properties inclusive of (1) a good heat resistance well in balance with oil resistance, (2) better low-temperature characteristic than acrylic rubber and (3) good weather resistance and ozone resistance. The ethylene-acrylic rubber also has a large mechanical strength, small compression permanent strain and good flexural resistance.

In addition to the above-mentioned conductivity-imparting agent, it is also possible to add a vulcanizer, a filler, an aging inhibitor, a promoter, or a processing aid, as desired, to the ethylene-acrylic rubber.

Examples of the filler for the ethylene-acrylic rubber may ordinarily include: carbon black, fumed colloidal anhydrous silica, calcium carbonate, barium sulfate, and titanium dioxide. However, other inorganic or organic fillers can also be added.

As the aging inhibitor, a diphenylamine-type or phenol-type anti-oxidant may ordinarily be used.

Chlorinated polyethylene is a thermoplastic polymer prepared by chlorinating polyethylene. Chlorinated polyethylene is rich in ozone resistance, softness, heat resistance, etc.

In addition to the above-mentioned conductivity-imparting agent, it is possible to add a stabilizer and various insulating fillers to the chlorinated polyethylene. Suitable examples of the stabilizer may include: ordinary organotin compounds, epoxy compounds, lead compounds, metallic soaps and metal oxide.

Epichlorohydrin-ethylene oxide rubber is formed by copolymerization of nearly equal mols of epichlorohydrin and ethylene oxide, and is a synthetic rubber having good heat resistance, cold resistance and ozone resistance in combination. The epichlorohydrin-ethylene oxide rubber used in the present invention may also include a ternary copolymer further including a small amount of alkyl glicidyl ether as a crosslinking monomer.

The above-mentioned binary and ternary copolymers have remarkably improved the low-temperature property which has been a defect of epichlorohydrin homopolymer.

In addition to the above-mentioned conductivity-imparting agent, it is also possible to add a vulcanizer, an aging inhibitor, a various insulating filler and a processing aid, as desired, to the epichlorohydrin-ethylene oxide rubber.

Chlorosulfonated rubber is a synthetic rubber developed by E. I. Dupont in 1951 and is obtained by reaction of polyethylene with chlorine and sulfuric acid gas. The chlorosulfonated polyethylene has a molecular structure as represented by the following formula:



Chlorosulfonated polyethylene has excellent ozone resistance, heat resistance, mechanical strength and wear resistance and also has small compression permanent strain.

Modified nitrile rubber is a blend rubber or a synthetic rubber developed for improving the poor ozone resistance of nitrile rubber (i.e., acrylonitrile-butadiene copolymer, NBR), and examples thereof may include a blend of nitrile rubber and polyvinyl chloride (NBR/PVC), a blend of nitrile rubber and EPDM (NBR/EPDM), hydrogenated nitrile rubber and carboxylated nitrile rubber, which are all commercially easily available.

Among the modified nitrile rubber, NBR/PVC can be obtained as a blend rubber showing advantageous properties comprising a compatible blend of NBR and PVC in almost any ratios because NBR and PVC have polar groups which are chemically similar to each other. Particularly, the NBR/PVC has remarkably improved ozone resistance and improved flexure resistance and wear resistance compared with NBR. Further, NBR/PVC has also improved extrusion processability compared with NBR and provides a shaped product having a surface which is smooth and shows a fine gloss.

NBR/EPDM is a blend rubber relatively recently developed in 1970's, has improved the ozone resistance of NBR by utilization of excellent ozone resistance of EPDM and also has good processability and mechanical properties.

Hydrogenated nitrile rubber is a rubber obtained by hydrogenating a large number of double bonds contained in the main chain of NBR (nitrile rubber) in a specific manner to lower the degree of unsaturation thereof, and has improved ozone resistance, heat resistance, cold resistance, mechanical strength, wear resistance and processability.

The contact charging member according to the present invention can assume any shape inclusive of those of a roller and a blade, which may be selected depending on a requirement of an electrophotographic apparatus for which it is adopted.

FIG. 1 is a schematic cross-sectional view of an embodiment of an electrophotographic apparatus including the contact charging member according to the present invention.

Referring to FIG. 1, a drum-type electrophotographic photosensitive member 1 is used as a charge-receiving member or charge-carrying member and comprises an electroconductive support layer 1b of, e.g., aluminum, and a photoconductive layer 1a formed on the support layer 1b. The photosensitive member 1 is rotated about an axis 1d at a prescribed peripheral speed in the clockwise direction. The photosensitive member 1 is uniformly charged by means of a roller-type charging member 2 for performing primary charging by contact to have prescribed polarity and potential at the surface thereof. The charging member 2 comprises a core metal (or a shaft) 2c as an electroconductive support, an elastic layer 2b and a surface layer 2d disposed in this order. The core metal 2c has both end sections at which the core metal is rotatably supported by a bearing member (not shown). The core metal 2c is disposed parallel to the axis 1d, and the charging member 2 is caused to abut upon the photosensitive member 1 under a prescribed pressure exerted by a pressing member (not shown), such as a spring, thus rotating mating with the rotation of the photosensitive member 1.

The primary charging is performed by applying a DC bias voltage or a superposition of a DC bias voltage and an AC bias voltage to the core metal 2c through a friction (or rubbing) electrode 3a by means of a power supply 3, thus contactively providing the peripheral surface of the rotating photosensitive member 1 with a prescribed polarity and a prescribed potential.

The peripheral surface of the photosensitive member 1 uniformly charged by the charging member 2 as described above is then subjected to imagewise exposure (e.g., laser beam scanning exposure or slit exposure of an original image) by image exposure means 10, whereby an electrostatic latent image corresponding to objective image data is formed on the peripheral surface of the photosensitive member 1. The thus formed latent image is developed or visualized by developing means 11 with a toner to form a toner image (or developed image) in sequence.

The toner image is successively transferred to the front side of a transfer-receiving material 14 such as paper, and is timely conveyed from a paper supply part (not shown) to a transfer position between the photosensitive member 1 and transfer means 12 (i.e., transfer roller in this embodiment) in synchronism with the rotation of the photosensitive member 1, by the transfer means 12. The transfer means (roller) 12 is used for charging the back side of the transfer-receiving material 14 so as to have a polarity opposite to that of the toner, whereby the toner image formed on the photosensitive member 1 is transferred to the front side of the material 14.

Then, the transfer-receiving material 14 having thereon the toner image is detached from the surface of the photosensitive member 1 and is conveyed to fixing means (not shown), whereby it is subjected to image fixing to be outputted as an image product.

The surface of the photosensitive member 1 after the transfer operation is subjected to cleaning by cleaning means 13 for removing and recovering an attached matter, such as a residual toner, from the surface of the photosensitive member 1, thus obtaining a cleaned surface to prepare for the next cycle.

In the present invention, a plurality of elements, such as a photosensitive member, a charging member, a developing means and a cleaning means, of an electrophotographic apparatus as shown in FIG. 1 can be integrally assembled to form a process cartridge, so that the cartridge may be detachably mountable to the apparatus main body. For example, the charging member according to the present invention and optionally one or both of the developing means and the cleaning means may be integrally assembled with the photosensitive member into a process cartridge, so that the cartridge may be attached to or detached from the apparatus body by the medium of a guiding means, such as a rail, of the apparatus body.

The charging member according to the present invention may be used as transfer means, primary charging means or discharge (or charge-removal) means, or further as a conveyor means, such as a paper supply roller.

The electrophotographic apparatus including the charging member according to the present invention may be embodied as a copying apparatus, a laser beam printer, an LED printer, or an electrophotography application apparatus, such as an electrophotographic plate-forming system.

Hereinbelow, the present invention will be described more specifically with reference to Examples, wherein "part(s)" means "part(s) by weight".

#### EXAMPLE 1

A roller member having an elastic layer was prepared in the following manner.

100 parts of EPDM ("EPT4045", mfd. by Mitsui Sekiyu Kagaku K.K.), 10 parts of zinc white No. 1 (valcanization promoter and reinforcing agent), 2 parts of stearic acid, 2 parts of promoter M (2-mercaptophenothiazole), 1 part of promoter BZ (zinc dibutyldithiocarbamate), 2 parts of sulfur, 5 parts of foaming agent ("CELLMIKE C", mfd. by Sankyo Kasei K.K.), 5 parts of foaming aid ("CELLTON NP", Sankyo Kasei K.K.), 20 parts of FEF (Fast Extrusion Furnace) carbon, 70 parts of insulating oil (paraffin oil), and 8 parts of electroconductive carbon ("ketjen black EC", mfd. by Lion K.K.) were blended and then kneaded for dispersion by a two-roller mill to form a rubber compound. The rubber compound was wound about an iron-made core metal preliminarily coated with a primer and then placed in a mold for pre-forming at 40° C. and 100 kg/cm<sup>2</sup> followed by vulcanization at 160° C. for 30 min. to form a roller member of a foam-type covered with a skin layer.

Then, the skin layer was removed by grinding with a grinder to complete a roller member having a core metal diameter of 6 mm, an outer diameter of 12 mm, a core metal length of 250 mm and an elastic layer length of 230 mm.

The resistance of the roller member was measured by placing the roller member on an aluminum sheet and put a load of 500 grams on each end to apply a total load of 1 kg to measure a resistance of 2×10<sup>6</sup> ohm.cm between the core metal and the aluminum sheet.

The roller member thus prepared was coated with a surface layer 2a (as shown in FIG. 1) by inserting the roller member into a preliminarily-formed non-heat-shrinkable tube of electroconductive polyethylene crosslinked by electron beam irradiation.

More specifically, an electroconductive polyethylene compound was prepared by blending 100 parts of high-pressure polyethylene ("SUNTEC LD L6810", mfd. by Asahi Kasei K.K.), 10 parts of a conductivity-imparting agent (carbon black "#4500", mfd. by Tohkai Carbon K.K.) and 2 parts of zinc stearate and melt-kneading the blend through an extruder to form a seamless tube product.

Then, the tube was irradiated with 200 M rad of electron beam at an accelerating voltage of 250 kV by means of an electron beam irradiator ("CURETRON", mfd. by Nissin High-voltage K.K.).

The thus-obtained electroconductive crosslinked non-heat-shrinkable polyethylene tube had an inner diameter of 11.5 mm, a thickness of 250  $\mu\text{m}$  and a volume resistivity of  $1 \times 10^6$ – $1 \times 10^8$  ohm.cm.

The above-prepared roller member was inserted into the non-heat shrinkable tube while blowing compressed air into the tube, thereby forming a surface layer (2a in FIG. 1) intimately fitting the circumference of the elastic layer of the roller member, thereby completing a charging roller.

The charging roller was incorporated in a process cartridge ("EP-L", available from Canon K.K.), which was mounted in a laser beam printer ("Laser Shot A404", mfd. by Canon K.K.) and subjected to a continuous image formation test of 10,000 sheets in respective environments of H/H (high temperature/high humidity of 32.5° C./80% RH), N/N (normal temperature/normal humidity of 25.0° C./50% RH) and L/L (low temperature/low humidity of 15.0° C./10% RH), whereby the resultant images gave the evaluation results shown in the following Table 1.

TABLE 1

| Environment  | H/H | N/N | L/L |
|--------------|-----|-----|-----|
| initial      | ○   | ○   | ○   |
| 3000 sheets  | ○   | ○   | ○   |
| 6000 sheets  | ○   | ○   | ○   |
| 10000 sheets | ○   | ○   | ○   |

The images were evaluated with eyes according to the following standard similarly as the results shown in Tables appearing hereinafter.

○: No images were accompanied with image defects, such as sanded fog, black spots and pinholes.

Δ: Nearly a half of the product images were accompanied with any one of the above-mentioned image defects.

x: Almost all of the product images were accompanied with any one of the above-mentioned image defects.

## EXAMPLE 2

An electroconductive nylon 12 compound was prepared in the same manner as in Example 1 except for using 100 parts of nylon 12 ("Diamide L1700", mfd. by Daicel Huels K.K.) in place of the polyethylene, additionally using 2 parts of triallyl isocyanurate (crosslinking aid) and changing the amount of the carbon black to 8 parts. Then, the compound was formed into a seamless tube in the same manner as in Example 1 except for changing the die temperature to 250° C. and was crosslinked by irradiation with 10 M rad of electron beam at an accelerating voltage of 150 kV.

The roller member prepared in Example 1 was inserted into the above prepared electroconductive crosslinked non-heat-shrinkable nylon 12 tube while blowing compressed air into the tube to complete a charging roller. As a result of continuous image formation in the same manner as in Example 1, the laser beam printer including the charging roller provided the evaluation results shown in the following Table 2.

TABLE 2

| Environment  | H/H | N/N | L/L |
|--------------|-----|-----|-----|
| initial      | ○   | ○   | ○   |
| 3000 sheets  | ○   | ○   | ○   |
| 6000 sheets  | ○   | ○   | ○   |
| 10000 sheets | ○   | ○   | ○   |

## EXAMPLE 3

An electroconductive ethylene-acrylic rubber compound was prepared in the following manner.

10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 94

manner as in Example 1, the laser beam printer including the charging roller provided the evaluation results shown in the following Table 4.

TABLE 4

| Environment  | H/H | N/N | L/L |
|--------------|-----|-----|-----|
| initial      | ○   | ○   | ○   |
| 3000 sheets  | ○   | ○   | ○   |
| 6000 sheets  | ○   | ○   | ○   |
| 10000 sheets | ○   | ○   | ○   |

## COMPARATIVE EXAMPLE 1

A charging roller was prepared in the same manner as in Example 1 except that the electroconductive polyethylene seamless tube after the formation thereof was directly subjected to the roller member insertion without the electron beam irradiation.

As a result of continuous image formation in the same manner as in Example 1, the laser beam printer including the charging roller provided the evaluation results shown in the following Table 5.

TABLE 5

| Environment | H/H | N/N | L/L |
|-------------|-----|-----|-----|
| initial     | ○   | ○   | ○   |
| 3000 sheets | ×   | ○   | ×   |
| 6000 sheets | ×   | ×   | ×   |

## COMPARATIVE EXAMPLE 2

A charging roller was prepared in the same manner as in Example 2 except that the electroconductive seamless tube after the formation thereof was directly subjected to the roller member insertion without the electron beam irradiation.

As a result of continuous image formation in the same manner as in Example 1, the laser beam printer including the charging roller provided the evaluation results shown in the following Table 6.

TABLE 6

| Environment  | H/H | N/N | L/L |
|--------------|-----|-----|-----|
| initial      | ○   | ○   | ○   |
| 3000 sheets  | ○   | ○   | ○   |
| 6000 sheets  | ○   | ○   | ○   |
| 10000 sheets | Δ   | ○   | ○   |

## COMPARATIVE EXAMPLE 3

A charging roller was prepared in the same manner as in Example 3 except that the electroconductive seamless tube after the formation thereof was directly subjected to the roller member insertion without the electron beam irradiation.

As a result of continuous image formation in the same manner as in Example 1, the laser beam printer including the charging roller provided the evaluation results shown in the following Table 7.

TABLE 7

| Environment | H/H | N/N | L/L |
|-------------|-----|-----|-----|
| initial     | ×   | ○   | ○   |
| 3000 sheets | ×   | ×   | ×   |
| 6000 sheets | ×   | ×   | ×   |

## COMPARATIVE EXAMPLE 4

A charging roller was prepared in the same manner as in Example 4 except that the electroconductive seamless tube after the formation thereof was directly subjected to the roller member insertion without the electron beam irradiation.

As a result of continuous image formation in the same manner as in Example 1, the laser beam printer including the charging roller provided the evaluation results shown in the following Table 8.

TABLE 8

| Environment | H/H | N/N | L/L |
|-------------|-----|-----|-----|
| initial     | ○   | ○   | ○   |
| 3000 sheets | ×   | ×   | ×   |
| 6000 sheets | ×   | ×   | ×   |

From the results shown in Tables 1-8, it is understood that the charging roller having a surface layer comprising a crosslinked polymer exhibits excellent durability and stably uniform charging ability suitable for electrophotographic image formation under various environmental conditions, thus being suitable for practical use.

Further, as a result of charging noise measurement, all the charging members in Examples 1-4 resulted in a noise below 55 dB, which is of practically no problem at all.

## EXAMPLE 5

A heat-shrinkable crosslinked seamless tube ("SUMITUBE G3", mfd. by Sumitomo Denko K.K.) comprising electroconductive chlorinated polyethylene was provided. The heat-shrinkable tube had an inner diameter of 16.5 mm and a thickness of 250  $\mu\text{m}$ .

Then, the roller member prepared in Example 1 was inserted into the heat-shrinkable tube, and the resultant combination was heated for 15 min. in a thermostat vessel at 250° C. having an air atmosphere to cause the tube to shrink about the elastic layer of the roller member, thereby completing a charging roller having an intimately attached surface layer.

The tube after the heat-shrinkage showed a volume resistivity of  $1 \times 10^6$ – $1 \times 10^8$  ohm.cm.

As a result of continuous image formation in the same manner as in Example 1, the laser beam printer including the charging roller provided the evaluation results shown in the following Table 9.

TABLE 9

| Environment | H/H | N/N | L/L |
|-------------|-----|-----|-----|
| initial     | ○   | ○   | ○   |
| 3000 sheets | ○   | ○   | ○   |
| 6000 sheets | ○   | ○   | ○   |

From the results shown in Table 9, it is understood that the charging roller having a surface layer comprising an elec-

troconductive crosslinked polymer exhibits excellent durability and stably uniform charging ability suitable for electrophotographic image formation under various environmental conditions, thus being suitable for practical use.

Further, as a result of charging noise measurement, the charging member of Example 9 resulted in a noise below 55 dB, which is of practically no problem at all.

#### EXAMPLE 6

100 parts alcohol-soluble nylon ("CM8000", mfd. by Toray K.K.) were dissolved in a methanol/water mixture solvent to form a vehicle solution having a solid content of 20 wt. %, to which 3 parts of a conductivity-imparting agent (carbon black "#4500", mfd. by Tohkai Carbon K.K.) and 2 parts of triallyl isocyanurate (crosslinking aid) were added and mixed for dispersion by a paint shaker, to obtain an electroconductive paint.

The roller member prepared in Example 1 was dipped in the electroconductive paint, taken out and dried to form a coating film about the roller member.

Then, the coating film on the roller member was irradiated with totally 10 M rad of electron beam by the electron beam irradiator used in Example 1. More specifically, the electron beam irradiation was repeated three times while changing the roller member direction so that the coating polymer was irradiated with a uniform dose of electron beam in the circumferential direction, to complete a charging roller having a surface layer (2a in FIG. 1) formed through the wet coating process.

As a result of continuous image formation in the same manner as in Example 1, the laser beam printer including the thus prepared charging roller provided the evaluation results shown in the following Table 10.

TABLE 10

| Environment  | H/H | N/N | L/L |
|--------------|-----|-----|-----|
| initial      | ○   | ○   | ○   |
| 3000 sheets  | ○   | ○   | ○   |
| 6000 sheets  | ○   | ○   | ○   |
| 10000 sheets | ○   | ○   | ○   |

#### COMPARATIVE EXAMPLE 5

A charging roller was prepared in the same manner as in Example 6 except that the triallyl isocyanurate was omitted from the electroconductive paint and the electron beam irradiation after the drying of the paint was also omitted.

As a result of continuous image formation in the same manner as in Example 1, the laser beam printer including the charging roller provided the evaluation results shown in the following Table 11.

TABLE 11

| Environment | H/H | N/N | L/L |
|-------------|-----|-----|-----|
| initial     | ○   | ○   | ○   |
| 3000 sheets | Δ   | Δ   | Δ   |
| 6000 sheets | ✗   | ✗   | ✗   |

#### EXAMPLE 7

An electroconductive paint was prepared by dissolving 100 parts of chlorinated polyethylene ("ELASREN

402ANA", mfd. by Showa Denko K.K.) in toluene to form a vehicle solution having a solid content of 5 wt. %, to which 30 parts of a conductivity-imparting agent (electroconductive tin oxide "SN-100", mfd. by Ishihara 5 Sangyo K.K.) was added and mixed for dispersion by a paint shaker.

A charging roller was prepared in the same manner as in Example 6 except for using the thus-prepared electroconductive paint.

10 As a result of continuous image formation in the same manner as in Example 1, the laser beam printer including the charging roller provided the evaluation results shown in the following Table 12.

TABLE 12

| Environment  | H/H | N/N | L/L |
|--------------|-----|-----|-----|
| initial      | ○   | ○   | ○   |
| 3000 sheets  | ○   | ○   | ○   |
| 6000 sheets  | ○   | ○   | ○   |
| 10000 sheets | ○   | ○   | ○   |

#### COMPARATIVE EXAMPLE 6

25 A charging roller was prepared in the same manner as in Example 7 except that the electron beam irradiation after the drying of the paint was omitted.

As a result of continuous image formation in the same 30 manner as in Example 1, the laser beam printer including the charging roller provided the evaluation results shown in the following Table 13.

TABLE 13

| Environment | H/H | N/N | L/L |
|-------------|-----|-----|-----|
| initial     | Δ   | ○   | ○   |
| 3000 sheets | ✗   | Δ   | Δ   |
| 6000 sheets | ✗   | ✗   | ✗   |

40 What is claimed is:

1. A contact charging member to be abutted against a charge-receiving member and supplied with a voltage for charging the charge-receiving member, comprising an electroconductive substrate, an elastic layer and a surface layer disposed in lamination; said surface layer comprising a crosslinked polymer crosslinked by irradiation with an electron beam.

2. A contact charging member according to claim 1, 45 wherein said surface layer comprises a seamless tube formed of the crosslinked polymer.

3. A contact charging member according to claim 1, wherein said surface layer has been formed by applying a coating film of a crosslinkable polymer and crosslinking the 55 coating film by electron beam irradiation.

4. A contact charging member according to claim 1, wherein said crosslinked polymer comprises crosslinked polyethylene.

5. A contact charging member according to claim 1, 60 wherein said crosslinked polymer comprises crosslinked nylon 12 or nylon 11.

6. A contact charging member according to claim 1, wherein said crosslinked polymer comprises crosslinked ethylene-acrylic rubber.

65 7. A contact charging member according to claim 1, wherein said crosslinked polymer comprises crosslinked polypropylene.

8. A contact charging member according to claim 1, wherein said crosslinked polymer comprises crosslinked chlorinated polyethylene.

9. A contact charging member according to claim 1, wherein said crosslinked polymer comprises crosslinked epichlorohydrin-ethylene oxide rubber.

10. A contact charging member according to claim 1, wherein said crosslinked polymer comprises crosslinked chlorosulfonated polyethylene.

11. A contact charging member according to claim 1, wherein said crosslinked polymer comprises crosslinked modified nitrile rubber.

12. A process for producing a contact charging member to be abutted against a charge-receiving member and supplied with a voltage for charging the charge-receiving receiving member, comprising the steps of:

- (1) forming an elastic layer on an electroconductive substrate,
- (2) shaping a polymer into a seamless tube,
- (3) crosslinking the polymer in the shape of the seamless tube by irradiation with an electron beam, and
- (4) covering the elastic layer with the crosslinked seamless tube.

13. An electrophotographic apparatus, comprising: a contact charging member and an electrophotographic photosensitive member; said contact charging member comprising an electroconductive substrate, an elastic layer and a surface layer disposed in lamination; said surface layer comprising a crosslinked polymer crosslinked by irradiation with an electron beam.

14. An electrophotographic apparatus according to claim 13, wherein said surface layer comprises a seamless tube formed of the crosslinked polymer.

15. A process cartridge detachably mountable to a main assembly of an image forming apparatus, comprising an electrophotographic photosensitive member and a charging member integrated with each other to form a cartridge, wherein the charging member comprises an electroconductive substrate, an elastic layer and a surface layer disposed in lamination; said surface layer comprising a crosslinked polymer crosslinked by irradiation with an electron beam.

16. A process cartridge according to claim 15, wherein said surface layer comprises a seamless tube formed of the crosslinked polymer.

\* \* \* \* \*

UNITED STATES PATENT AND TRADEMARK OFFICE  
**CERTIFICATE OF CORRECTION**

PATENT NO. : 5,625,858

DATED : April 29, 1997

INVENTORS : YOSHIRO HIRAI ET AL.

Page 1 of 3

It is certified that error appears in the above-identified patent and that said Letters Patent is hereby corrected as shown below:

ON TITLE PAGE ITEM:

[56] Foreign Patent Documents

"63-167380 3/1988 Japan" should read --63-167380 7/1988  
Japan--.

COLUMN 2

Line 35, "in-environmental" should read --in  
environmental--.

COLUMN 4

Line 20, "obtained" should read --obtained by--;  
Line 27, "of" should read --of a--.

COLUMN 5

Line 36, "is" should read --is more--;  
Line 38, delete "of";  
Line 40, "and" should read --and there is--;  
Line 41, "treatment, and than the" should read  
--treatment. Further, the electron beam  
crosslinking is better than the--;

UNITED STATES PATENT AND TRADEMARK OFFICE  
**CERTIFICATE OF CORRECTION**

PATENT NO. : 5,625,858

DATED : April 29, 1997

INVENTORS : YOSHIRO HIRAI ET AL.

Page 2 of 3

It is certified that error appears in the above-identified patent and that said Letters Patent is hereby corrected as shown below:

COLUMN 5

Line 62, "it" should read --at--.

COLUMN 7

Line 43, "remarkably" should read --remarkable--;  
Line 45, "comprise" should read --comprises--.

COLUMN 8

Line 39, "blend" should read --blended--;  
Line 48, "blend" should read --blended--;  
Line 59, "in 1970's," should read --(in the  
1970's),--.

UNITED STATES PATENT AND TRADEMARK OFFICE  
**CERTIFICATE OF CORRECTION**

PATENT NO. : 5,625,858

DATED : April 29, 19997

INVENTORS : YOSHIRIHO HIRAI ET AL.

Page 3 of 3

It is certified that error appears in the above-identified patent and that said Letters Patent is hereby corrected as shown below:

COLUMN 11

Line 36, "with eyes" should read --visually--.

COLUMN 17

Line 15, "receiving" (second occurrence) should be deleted.

Signed and Sealed this  
Second Day of December, 1997

Attest:



BRUCE LEHMAN

Attesting Officer

Commissioner of Patents and Trademarks